

Feb. 3, 1970

C. B. HAEGERT

3,493,034

METHOD OF MAKING AN ELECTRICAL CONNECTOR

Filed March 6, 1968

*Fig. 1.*



*Fig. 2.*



*Fig. 3.*



*Fig. 5.*



INVENTOR  
Clarence B. Haegert

BY *Shumaker and Mattare*  
ATTORNEYS

## 1

3,493,034

### METHOD OF MAKING AN ELECTRICAL CONNECTOR

Clarence B. Haegert, P.O. Box 318,  
Coffeyville, Kans. 67337  
Filed Mar. 6, 1968, Ser. No. 710,829  
Int. Cl. B22d 23/00

U.S. Cl. 164—47

9 Claims

### ABSTRACT OF THE DISCLOSURE

The method of the present invention includes the steps of providing a zinc base alloy including aluminum, copper, magnesium, iron, lead, cadmium, tin and zinc within certain critical ranges, heating the alloy to a molten state, and then casting the molten alloy to form an electrical connector including a body means having means for securing an electrical member thereto. The casting step of the method comprises either a sandcasting procedure or a die casting procedure.

### BACKGROUND OF THE INVENTION

The present invention relates to electrical connectors of various types. Electrical connectors of this type including means for securing an electrical member thereto have in the past been generally formed of a brass-lead alloy or a copper alloy. Such prior art connectors are relatively expensive and are subject to excessive corrosion. This excessive cost arises due to the materials employed in the connectors as well as the method of making the connectors.

### SUMMARY OF THE INVENTION

The present invention comprises an electrical connector wherein the body means thereof is formed of a zinc base alloy. The utilization of the zinc base alloy of the present invention substantially reduces the cost of the connector since the materials involved are cheaper, and furthermore the connector can be readily manufactured.

In the present invention, the method includes the step of sandcasting or die casting the electrical connector, and this provides a most practical and economical manner of manufacturing an electrical connector of this type.

Also, surprisingly enough, it has been found that electrical connectors made of such a zinc base alloy according to the present invention have better electrical conductivity than prior art connectors made of a brass-lead alloy or a copper alloy, and also exhibit good tensile strength. Additionally, the connector of the present invention has very good resistance to corrosion.

### BRIEF DESCRIPTION OF THE DRAWING

FIG. 1 is a top perspective view illustrating a first form of electrical connector according to the present invention;

FIG. 2 is a top perspective view illustrating a second form of electrical connector according to the present invention;

FIG. 3 is a top perspective view of a further electrical connector according to the present invention;

FIG. 4 is a top perspective view of still another electrical connector according to the present invention; and

FIG. 5 is a top perspective exploded view of the structure illustrated in FIG. 4.

### DESCRIPTION OF THE PREFERRED EMBODIMENTS

Referring now to the drawings wherein like reference characters designate corresponding parts throughout the several views, a first form of electrical connector is illus-

## 2

trated in FIG. 1 wherein the connector is indicated generally by reference numeral 12.

This connector includes a body means 14 having an integral hollow cylindrical portion 16 for receiving an electrical cable or the like. The body means also includes a pair of spaced integral leg portions 18 and 20 having a tapered bore 24 defined therein for receiving a battery terminal whereby the device is adapted to operate as a conventional battery terminal connector.

10 A bolt 30 extends through aligned holes provided in the outer ends of arms 18 and 20, the bolt 30 having an enlarged head portion 32 received within a cutout 34 provided in leg portion 20 of the body means. A nut 36 is threaded on the far end of the bolt as seen in FIG. 1 for clamping the connector on a battery terminal.

15 A small screw 40 is adapted to be threaded into a tapped hole provided in enlarged head 32 for securing a lug 42 to the connector. This lug has a suitable hole provided therein for receiving the threaded shank portion of screw 40. The end portion 44 of lug 42 is hollow for receiving a suitable electrical member which is crimped thereto.

20 A threaded stud 50 extends upwardly from portion 16 of the connector and has a tapped hole formed therein for receiving a small screw 52 which is employed for holding lug 54 in place, lug 54 being of substantially the same construction as lug 42.

25 Referring now to FIG. 2 of the drawing, a modified electrical connector is indicated generally by reference numeral 60 and may also comprise a battery terminal connector. This connector includes a body means 62 having a hollow cylindrical portion 64 for receiving an electrical cable or the like. The body means also includes a pair of spaced leg portions 66 and 68 having aligned holes 70 and 72 formed therethrough for receiving a suitable nut and bolt assembly for clamping the connector on a battery terminal.

30 A tapered bore 75 is formed between spaced legs 66 and 68 for receiving a conventional battery terminal.

35 Referring now to FIG. 3, a further modified form of electrical connector according to the present invention is illustrated. The electrical connector is indicated generally by reference numeral 80 and includes a body means including a flat end portion 82 having a hole 84 formed therethrough. The opposite end portion 86 of the body means is of generally cylindrical configuration and is hollow for receiving a cable or the like, the bared end of the cable being crimped in position within such hollow end portion of the body means.

40 Referring now to FIGS. 4 and 5, a still further modified form of electrical connector is illustrated. The connector is indicated generally by reference numeral 90 and includes a three-part body means, the body means including a bolt 92 having an enlarged hex head 94 at one end thereof and having a longitudinally extending slot 96 formed therein. The external portion of the lower part of the bolt is provided with threads 98.

45 The body means includes an intermediate member 100 the main portion of which is adapted to slide within the slot 96 formed in bolt 92. Member 100 includes depending leg portions 102 and 104 which are spaced apart and which are adapted to be inserted through a threaded bore 106 provided in a nut 108 and then turned upwardly as indicated in phantom lines in FIG. 5 so as to retain members 100 and 108 in assembled relationship as seen in FIG. 4. The threaded bore 106 is adapted to be threaded on the external threads 98 provided on the bolt 92.

50 As seen most clearly in FIG. 5, the upper surface of member 100 is provided with a central generally V-shaped groove 110. A pair of lugs 112 extend outwardly in opposite directions from one end of member 100, and a similar pair of lugs 114 extend outwardly in opposite di-

tions from the opposite end of member 100. The portion of member 100 between lugs 112 and 114 is adapted to fit within the slot 96 provided in bolt member 92, lugs 112 and 114 serving to retain member 100 in position and guide its movement in a vertical direction as seen in drawings.

It is apparent that when the electrical connector is in the embled relationship shown in FIG. 4, rotation of nut 3 with respect to bolt 92 will cause member 100 to be rotated and lowered within the slot 96 in the bolt member thereby a suitable electrical member may be clamped between the upper surface of member 100 and the under-surface of the hex head 94 of the bolt.

The body means of each of the electrical connectors described in connection with FIGS. 1 through 5 inclusive is formed of a zinc base alloy having a particular composition.

The following three examples represent compositions of the table for use as the body means of an electrical connector according to the present invention.

#### EXAMPLE I

|          | Percent             |
|----------|---------------------|
| uminum   | 3.9-4.3.            |
| pper     | .75-1.25.           |
| agnesium | .03-.06.            |
| on       | Up to .075 maximum. |
| ad       | Up to .003 maximum. |
| idmium   | Up to .003 maximum. |
| n        | Up to .002 maximum. |
| nc       | Balance.            |

#### EXAMPLE II

|          | Percent             |
|----------|---------------------|
| uminum   | 3.5-4.5.            |
| pper     | 2.5-3.5.            |
| agnesium | .02-10.             |
| on       | Up to .100 maximum. |
| ad       | Up to .007 maximum. |
| idmium   | Up to .005 maximum. |
| n        | Up to .005 maximum. |
| nc       | Balance.            |

#### EXAMPLE III

|          | Percent             |
|----------|---------------------|
| uminum   | 3.9-4.3.            |
| pper     | Up to .10 maximum.  |
| agnesium | .03-0.6.            |
| on       | Up to .075 maximum. |
| ad       | Up to .003 maximum. |
| idmium   | Up to .003 maximum. |
| n        | Up to .002 maximum. |
| nc       | Balance.            |

In each of the above examples, the percentages are by weight of the composition, and it will be noted that in each case the major portion of the composition comprises zinc which is the balance of the composition in each of the three examples.

In carrying out the method of the present invention, one of the aforementioned zinc base alloys is provided and heated until it is in a molten state. The molten metal is then either sandcast or die cast to form one or more components of the electrical connector which includes body means having means for securing an electrical member thereto.

It is apparent from the foregoing that there is provided a new and novel method of making an electrical connector body means having means for securing an electrical connector member thereto and wherein the body means is formed of a zinc base alloy which enables the connector to be manufactured at a lower cost with good electrical conductivity, good tensile strength, and good corrosion resistance characteristics.

As this invention may be embodied in several forms without departing from the spirit or essential characteristics thereof, the present embodiment is therefore illustrative and not restrictive, and since the scope of the invention is defined by the appended claims, all changes that fall within the metes and bounds of the claims or that form their functional as well as conjointly cooperative equivalents are therefore intended to be embraced by those claims.

10 I claim:

1. The method of making an electrical connector comprising providing a zinc base alloy consisting essentially of about 3.9 to 4.3% aluminum, about .75 to 1.25% copper, about .03 to .06% magnesium, up to about 15 .075% iron, up to about .003% lead, up to about .003% cadmium, up to about .002% tin, the balance being zinc, all of said percentages being by weight of the composition, heating said alloy until it is in a molten condition, and then casting said molten alloy to form an electrical 20 connector including a body means having means for securing an electrical member thereto.

2. The method as defined in claim 1 wherein said casting step is a sandcasting procedure.

25 3. The method as defined in claim 1 wherein said casting step is a die casting procedure.

4. The method of making an electrical connector comprising providing a zinc base alloy consisting essentially of about 3.5 to 4.5% aluminum, about 2.5 to 3.5% copper, about .02 to .10% magnesium, up to about .100% iron, up to about .007% lead, up to about .005% cadmium, up to about .005% tin, the balance being zinc, all of said percentages being by weight of the composition, heating said alloy until it is in a molten condition, and then casting said molten alloy to form an electrical 30 connector including a body means having means for securing an electrical member thereto.

35 5. The method as defined in claim 4 wherein said casting step is a sandcasting procedure.

40 6. The method as defined in claim 4 wherein said casting step is a die casting procedure.

45 7. The method of making an electrical connector comprising providing a zinc base alloy consisting essentially of about 3.9 to 4.3% aluminum, up to about .10% copper, .03 to 0.6% magnesium, up to about .075% iron, up to about .003% lead, up to about .003% cadmium, up to about .002% tin, the balance being zinc, all of said percentages being by weight of the composition, heating said alloy until it is in a molten condition, and then casting said molten alloy to form an electrical 50 connector including a body means having means for securing an electrical member thereto.

55 8. The method as defined in claim 7 wherein said casting step is a sandcasting procedure.

9. The method as defined in claim 7 wherein said casting step is a die casting procedure.

#### References Cited

##### FOREIGN PATENTS

60 21,525 2/1935 Australia.

##### OTHER REFERENCES

Materials and Methods, Cast Zinc Alloys, number 199, October, 1950, p. 91., New Jersey Zinc Co.

65 Zamar Alloys for Zinc Alloy Die Castings, a technical department Bulletin, E. A. Anderson and G. L. Werley, New Jersey Zinc Company, 160 Front Street, New York 7, New York, 1944.

70 J. SPENCER OVERHOLSER, Primary Examiner

J. E. ROETHEL, Assistant Examiner

U.S. Cl. X.R.

164—113; 339—278